

# UNITED STATES PATENT OFFICE.

OZIAS DODGE, OF NORWICH, CONNECTICUT.

## PROCESS OF PRODUCING MECHANICAL NEGATIVES.

1,120,913.

Specification of Letters Patent. Patented Dec. 15, 1914.

No Drawing.

Application filed April 18, 1912. Serial No. 691,741.

*To all whom it may concern:*

Be it known that I, OZIAS DODGE, a citizen of the United States of America, residing at Norwich, in the county of New London and State of Connecticut, have invented new and useful Improvements in Processes of Producing Mechanical Negatives, of which the following is a description.

This invention relates to the production 10 of photographically opaque and transparent negatives from a positive drawing or printed impression, for example, without the use of a photographic plate; and the objects of my invention are: 1st. To transform a drawing, with all its gradations of shading, into a photographically opaque stencil or negative, which gives all the delicacy and detail of the original. 2nd. To provide to photo engravers, artists and lithographers new 20 means for producing printing surfaces upon copper, zinc, lithographic stone, and the like, and to produce printing surfaces electrolytically built up, without the use of a camera. 3rd. To preserve a faithful negative of 25 original drawings or printed impressions for indefinite further uses.

My invention consists in transforming a drawing or printed impression made upon a transparent surface, such as the film patented to me December 24, 1907, so that it 30 shall become a photographically opaque negative.

Prior to my invention there was no method of obtaining a negative except by 35 using a photographic plate, whereas by my present invention the surface bearing the drawing or printed image becomes the negative, and in the place of the drawing there are transparent lines upon an opaque 40 ground; and here my invention ends, but the uses of this negative in producing printing surfaces for the photo engraver, for artists, and for lithographers, and in producing relief plates built up electrolytically, 45 will at once be seen and appreciated by those skilled in the art.

I will now describe my improved process in its best form as now practised by me.

The starting materials are, preferably, a 50 grained gelatin film, of a coarse, velvet or medium grain best suited to the nature of the drawing, and a pencil or ink especially prepared, which is soluble in gasolene or similar liquids, and insoluble in alcohol or

water. On the grain side of this film the 55 drawing is executed with such pencil or ink, and should show a grain in all parts except the deep black, and high lights should be taken out with a scraper. I prefer not to use a rubber, but to erase with a cloth moistened with gasolene if extensive erasures are needed, or to clean off the entire drawing. The completed drawing is like any other drawing, only resting on a transparent support, and can be best judged by laying it 65 face down upon white and looking at it from the back.

In the case of printed impressions, proofs are printed as guides in adding work for the production of several plates for color printing, thereby insuring a register as they are identical except for the individual work on or around the proof. These proofs are printed upon the film above mentioned in an ink soluble in gasolene or similar liquids 70 if the printed image is to become the transparency with the additions and work upon them, or in an ink not soluble in the above liquids if they are only to serve as guides in laying in the original work to make the 75 various plates for color printing. As the proofs and work upon them are on a transparent film they can be laid one over the other to advantage to judge how the final picture will be built up from the various plates. 80 This drawing or printed impression is now 85 to be converted into a reverse printing negative for the sensitized zinc or copper plate, by covering the face of the drawing and the film supporting it with a photographically 90 opaque varnish, composed preferably of a solution of shellac and alcohol, to which I add red and yellow dyes, making it opaque to actinic rays of light. This varnish is so balanced hygroscopically that it unites to a 95 slight depth with the film, rendering it opaque to actinic light and covers the drawing as well as the face of the film supporting it. The drawing should be dusted off before applying the varnish, and no varnish should 100 be allowed to run onto the under side of the film. In small work, the varnish may be applied by flowing; or if the drawing is large, or difficulty is experienced in flowing it, the drawing may be varnished with a 105 thick camel hair or water-color brush well loaded with varnish, by beginning at the top and carrying as wide a band of color as

the brush will allow straight across, the second stroke just overlapping the lower edge of the first, and continuing thus to the bottom. I then dry the varnish, warming 5 the film slightly while drying, and this stage may occupy from three to five minutes.

When dry I lay the film flat upon clean paper and rub the surface lightly with a cloth or cotton moistened with gasolene or 10 similar liquids, by which the drawing or printed proof is removed, leaving a red film stencil or photographic printing negative; and with the production of this negative, my present process is complete.

15 I will now describe the specially prepared ink which I prefer to use, and the special pencil which I prefer to use in making the drawing above referred to. The ink is composed of tallow, wax, soap and shellac in 20 about equal parts, to which is added a fine Paris block for color. This ink is cast into sticks and in use is rubbed up with water as with lithographic writing ink. The pencils are composed of similar materials with a 25 larger proportion of wax, or ordinary lithographic pencils can be used.

The formula and directions for making the varnish are as follows: 32 ounces grain 30 alcohol, 2 ounces dry shellac, common brown shellac suffices. These I shake well together and allow them to stand from three to four days. The clear liquid is then decanted off from the precipitate. To 32 ounces of the liquid are added one ounce of water, 300 35 grains of auramin, soluble in alcohol, yellow dye, and 280 grains of rhodamin, soluble in alcohol, red dye. When the color is finally dissolved, the solution is filtered and is then ready for use as above described; giving if 40 applied under the foregoing directions, a perfectly even color, opaque to the actinic rays of light, and the drawing will remain undisturbed. Thus, by a single operation, without photography, the drawing itself be- 45 comes by my process the transparent negative printing black lines upon a white ground. It retains its original dimensions, shows all the gradations of shading of the original drawing, transposed as faithfully 50 as by any of the known photographic methods. The parts covered by the opaque varnish hold back the light from a sensitized surface, while the drawing being now a transparency, prints in exact ratio to the 55 amount of pencil used in making it. But by this method, instead of the usual pen and ink effect of a line cut, all the delicacy of shading, from white to deep black, is pre- 60 served in the reproduction, and in making it pen and pencil can be used on the same drawing.

The opaque solution thus described, and which is mentioned in the claims, is a dye of a deep ruby color, opaque to actinic rays. 65 The particular characteristics of the opaque

solution are that it penetrates the substance of the drawing sparingly, passing through the lighter portions of the drawing to the film underneath, which it readily penetrates. This penetration through the drawing, and 70 into the film, is due to the small percentage of water in the alcohol, which makes a solvent which will penetrate this particular ink or pencil composing the drawing, in ratio to the density of the drawing, and this solution which thus penetrates to the film penetrates into the film in this ratio to the density of the drawing. The percentage of water may vary from three to fifteen per cent. of the whole solution, but without 75 water in some appreciable percentage, I have not observed hitherto that I can get penetration of the film by the solution in ratio to the density of the drawing.

I have described the method, the film employed, the ink and pencil, the varnish, and the various steps by way of illustration only, and not as limitations, from which there may be variations without departing from the spirit of my invention; and I use the word drawing in both this specification and the following claims to designate any picture, lines, shadings or characters made upon a film by handwork or by any process of printing, or by transferring or photographing the same on the film with a substance which may be removed by a suitable solvent, leaving in its place a transparency, and especially if such transparency may be graduated as to degree of transparency to 95 correspond with the density of the drawing; and I especially contemplate this improved process as applicable to such drawings on the grained gelatin films patented to me as aforesaid, when treated so that they become 100 with the drawing upon them, transparent printing negatives.

Having now described my invention, what I claim as new and desire to secure by Letters Patent is:

1. The process of producing negatives, which consists in producing a drawing upon a transparent film, treating the same with an opaque solution, which renders the surface bearing the drawing opaque, and leaves the drawing unaltered, but penetrates the drawing in proportion to the density thereof, and penetrates the film underneath the drawing in ratio to the density of the drawing; removing the drawing by a solvent, and leaving in its place a transparency graduated as to degree of transparency corresponding to the density of the drawing.

2. The process of producing negatives, which consists in printing an image in greasy ink upon a transparent film, treating the same with an opaque solution, which renders the surface bearing the printed image opaque and leaves the proof unaltered, but penetrates the proof in propor-

tion to the density thereof, and penetrates the film underneath in ratio to the density of the proof, removing the proof by a solvent, leaving in its place a transparency graduated as to degree of transparency corresponding to the density of the proof.

In witness whereof, I have hereunto set

my hand and affixed my seal, at Norwich, in the county of New London, and State of Connecticut, this 12th day of April, 1912.

OZIAS DODGE. [L. S.]

In presence of—

G. A. THOMPSON,

JOHN P. HUNTINGTON.